

1

3,677,765

## SILVER HALIDE SUPERSENSITIZED PHOTOGRAPHIC EMULSION

Yoshiyuki Nadazawa, Yashuharu Nakamura, Haruo Takei, Akira Sato, and Tadashi Ikeda, Minami-Ashigara-machi, Kanagawa, Japan, assignors to Fuji Photo Film Co., Ltd., Minami-Ashigara-machi, Kanagawa, Japan

No Drawing. Filed Feb. 10, 1971, Ser. No. 114,338  
Claims priority, application Japan, Feb. 10, 1970,

45/11,586

Int. Cl. G03c 1/14

U.S. Cl. 96—124

7 Claims

### ABSTRACT OF THE DISCLOSURE

A silver halide light-sensitive photographic emulsion containing a combination of at least one sensitizing dye represented by the following Formula I and at least one sensitizing dye represented by the following Formula II:



wherein  $R_1$  and  $R_2$  each represents a lower alkyl group or a substituted lower alkyl group,  $Z_1$  and  $Z_2$  each represents an atomic group necessary to complete a benzothiazole nucleus, a benzoselenazole nucleus or a naphthothiazole nucleus,  $X_1$  represents an anion, and  $n$  represents 0 or 1,  $n=0$  when an intra-molecular salt is formed;



wherein  $R_5$  represents a lower alkyl group and  $R_3$ ,  $R_4$ ,  $Z_3$ ,  $Z_4$ ,  $X_2$  and  $m$  each has the same meaning as  $R_1$ ,  $R_2$ ,  $Z_1$ ,  $Z_2$ ,  $X_1$  and  $n$  respectively.

### BACKGROUND OF THE INVENTION

#### Field of the invention

The present invention relates to a spectrally sensitized silver halide light-sensitive photographic emulsion and especially to a silver halide light-sensitive photographic emulsion in which at least two sensitizing dyes are used in combination, by which a wavelength region spectrally sensitized by each sensitizing dye is super-sensitized and a high red-sensitivity is obtained.

#### Description of the prior art

In photographic light-sensitive materials commonly used, various spectral sensitivity distributions are required corresponding to the object being photographed. In the photographic light-sensitive material art, a method is well known whereby a certain kind of sensitizing dye is added to the silver halide emulsion to expand its sensitive wavelength range to a further long wavelength range; that is, a spectral sensitization technique.

In general, two or more kinds of sensitizing dyes are used together in the photographic sensitive material in

2

order to obtain a desired spectral sensitivity distribution. However, in many cases, the spectral sensitivity resulting by using two or more sensitizing dyes together, to adjust the spectral sensitivity distribution, is lower than that obtained by using each sensitizing dye by itself. However, in certain cases, the spectral sensitizing function obtained by the use of a sensitizing dye having a limited chemical structure may be additionally strengthened by using it together with another sensitizing dye or organic compound having a certain limited chemical structure. This phenomenon is known as a supersensitization function.

An object of the present invention is to provide a silver halide photographic light-sensitive emulsion having a high red-sensitivity in a spectral sensitized wavelength range of 620–690 nm. by using two different kinds of sensitizing dyes in combination. This wavelength range is a spectral wavelength range used widely in black and white sensitive materials or in color photographic red-sensitive layers.

### SUMMARY OF THE INVENTION

The above-mentioned object of the present invention has been attained by using a combination of sensitizing dyes represented by the following Formulae I and II in a photographic silver halide light-sensitive emulsion:



wherein  $R_1$  and  $R_2$  each represents a lower alkyl group (for example, methyl or ethyl, etc.) or a substituted alkyl group commonly used in sensitizing dyes (for example, a  $\gamma$ -sulfopropyl group, a  $\gamma$ -sulfobutyl group, a  $\delta$ -sulfobutyl group, a  $\beta$ -hydroxyethyl group, a  $\beta$ -carboxy propyl group, a  $\delta$ -carboxybutyl group or an allyl group, etc.);  $Z_1$  and  $Z_2$  each represents an atomic group necessary to complete a benzothiazole nucleus, a benzoselenazole nucleus or a naphthothiazole nucleus, wherein the nucleus may be substituted with, for example, a halogen atom (for example, chlorine or bromine, etc.), a lower alkyl group, a hydroxyl group, an alkoxy group (for example, methoxy or ethoxy, etc.), a phenyl group, a carboxyl group, or an alkoxy-carbonyl group (for example, methoxycarbonyl or ethoxycarbonyl, etc.);

$X_1^-$

represents an anion of the type normally used in cyanine dyes (for example, a chlorine, bromine, iodine, p-toluenesulfonic acid or an ethylsulfonic acid ion, etc.); and  $n=0$  or 1,  $n=0$  when an intra-molecular salt is formed; and



wherein  $R_5$  represents a lower alkyl group (for example, methyl or ethyl, etc.),  $R_3$  and  $R_4$  each represents a lower alkyl group (for example, methyl or ethyl, etc.) or a substituted alkyl group (for example,  $\gamma$ -sulfopropyl,  $\gamma$ -sulfobutyl,  $\delta$ -sulfobutyl,  $\beta$ -hydroxypropyl,  $\beta$ -carboxyethyl or allyl, etc.),  $Z_3$  and  $Z_4$  each represents a group of atoms necessary to form a benzothiazole nucleus, a benzoselenazole nucleus or a naphthothiazole nucleus, wherein the

3

nucleus may be substituted with, for example, a halogen atom (for example, chlorine or bromine, etc.), a lower alkyl group (for example, methyl, ethyl, propyl, etc.) an alkoxy group (for example, methoxy or ethoxy, etc.), an aryl group (for example, phenyl, etc.), a hydroxyl group, a carboxyl group, or an alkoxy carbonyl group (for example, methoxycarbonyl or ethoxycarbonyl, etc.);

xii

represents an anion of the type normally used in cyanine dyes (for example, a chlorine, bromine, iodine, p-toluenesulfonic acid or ethylsulfonic acid ion, etc.);  $m$  represents 0 or 1,  $m$  being 0 when an intra-molecular salt is formed.

A characteristic of the sensitizing dye represented by Formula I (hereinafter termed sensitizing dye (I)) is that the hydrogen atom at the  $\beta$ -position of the methine chain of the cyanine dye containing a benzothiazole nucleus, a benzoselenazole nucleus or a naphthothiazole nucleus is replaced with a phenylethyl group. Such cyanine dyes easily form an optical (color) sensitization range which has a comparatively easy inclination at the long wavelength side of the maximum sensitization part. On the other hand, the cyanine dyes represented by Formula II (hereinafter termed sensitizing dye (II)) easily form an optical (color) sensitization range which has a comparatively steep inclination at the long wavelength side of the maximum sensitization part. A high red-sensitivity can be obtained by using a combination of sensitizing dyes (I) and (II) as compared with the cases of using each sensitizing dye by itself. Further, it is possible to use the dyes together with an optical sensitizer in order to increase the green-sensitivity (a pseudocyanine dye, etc.) or other optical sensitizers having other spectral sensitization ranges.

The following compounds are examples of sensitizing dyes which may be used in the present invention. However, the sensitizing dyes shown below are merely given as examples, applicants having no intention of being limited thereto.

(I)

A



B



6



8



10



25



6



E



II



75



The sensitizing dyes represented by Formulae I and II used in the present invention can be produced by any known method.  
 For example, they can be easily synthesized by those skilled in the art with reference to U.S. Pat. No. 2,503,776, German patent specification No. 929,080 or German patent specification No. 1,072,765.

Namely, the sensitizing dyes represented by Formula I are prepared by reacting a compound represented by Formula III:



wherein  $Z_1$ ,  $R_1$ ,  $X_1$  and  $n$  have the same meaning as in Formula I, and  $R'$  represents an alkyl group (for example, methyl or ethyl, etc.), with a compound represented by Formula IV:



wherein  $Z_2$ ,  $R_2$ ,  $X_1$  and  $n$  have the same meaning as in Formula I, in a suitable solvent such as methanol, ethanol or isopropanol in the presence of a basic condensing agent such as triethylamine under refluxing by heating.

The term "lower alkyl group" indicates an alkyl group having 1-5 carbon atoms.

The physical properties of the typical examples of the sensitizing dyes (I) shown above are as follows:

| Dye No. | M.P. (° C.) | $\lambda_{\text{max.}}$<br>(nm.) |
|---------|-------------|----------------------------------|
| I-A     | 281         | 559                              |
| I-B     | 288         | 564                              |
| I-C     | 269         | 558                              |
| I-D     | 268         | 563                              |
| I-E     | 297         | 577                              |
| I-F     | 257         | 555                              |
| I-G     | 222         | 533                              |
| I-H     | 280         | 558                              |
| I-I     | > 300       | 558                              |
| I-J     | 257         | 558                              |
| I-K     | 246         | 558                              |
| I-L     | 258         | 664                              |
| I-M     | 288         | 562                              |

The spectral sensitization method of the present invention is effective for spectrally sensitizing gelatino silver halide photographic emulsions. Further, it is possible to sufficiently sensitize emulsions containing a hydrophilic colloid, excepting gelatin, such as agar-agar collodion, water-soluble cellulose derivatives, polyvinyl alcohol and other synthetic or natural hydrophilic resins by this method.

As the photographic emulsion used in the present invention, mixed silver halide emulsions such as of silver iodide bromide and silver chloroiodo bromide are suitable.

In order to adjust the spectral sensitized photographic emulsion of the present invention, sensitizing dyes (I) and (II) may be admixed with the photographic emulsion by any common method. In practice, coloring material is usually added as a solution in a suitable solvent such as methanol or ethanol to the emulsion. The amount of sensitizing dyes (I) or (II) is preferably within the range of from  $10^{-6}$  mole to  $10^{-3}$  mole of dye per mole of silver halide.

The molar ratio of sensitizing dye (I) to dye (II) used in the emulsion can vary over a wide range of 9:1-1:9 according to the desired effect.

The photographic emulsion of the present invention can be subjected to hypersensitization and supersensitization by any well known method. In the preparation of the photographic emulsion of the present invention, additives commonly used such as sensitizers, stabilizers, color controlling agents, hardeners, surface active agents, antifogging agents, plasticizers, development accelerators, color

formers or whitening fluorescent agents, etc., can be added to the emulsion by usual methods.

The photographic emulsion of the present invention can be applied to a suitable support such as glass, films of cellulose derivatives, synthetic resin films and baryta paper by any common method.

The following examples further illustrate the present invention.

Silver halide photographic emulsions were prepared by adding the above-mentioned sensitizing dyes (I) and (II) individually to a silver iodide bromide emulsion

$$(\text{AgI:AgBr} = 7 \text{ moles:93 moles})$$

On the other hand, silver halide photographic emulsions which contain a combination of sensitizing dyes (I) and (II) were prepared. After applying these emulsions to triacetyl cellulose film bases and drying, the resulting films were exposed to a 64-lux daylight lamp (corresponding to 5400° K.) as the light source through a Fuji No. 7 filter (trademark) (red filter through which rays having a long wavelength of about 580 nm. penetrate, produced by Fuji Photo Film Co., Ltd.) and subjected to development. As the developing solution, that having a composition described in Table 1 was used.

TABLE 1

|                         | G.  |
|-------------------------|-----|
| Metol                   | 2   |
| Sodium sulfite          | 100 |
| Hydroquinone            | 5   |
| Borax                   | 2   |
| Water to make, 1 liter. |     |

Table 2 shows the red sensitivity and maximum sensitization achieved employing the above-mentioned sensitizing dye (I) by itself. Table 3 shows the red sensitivity and maximum sensitization realized when using the above-mentioned sensitizing dye (II) by itself. Table 4 shows the red sensitivity and maximum sensitization realized when using combinations of sensitizing dyes (I) and (II).

TABLE 2

| Dye No. | Amount of sensitizing dye (10 <sup>-5</sup> mols/kg. emulsion) (ml.) | Emulsion | Maximum sensitization (nm.) | Red sensitivity |
|---------|----------------------------------------------------------------------|----------|-----------------------------|-----------------|
| A       | 8                                                                    | AgBr/I   | 634                         | 203             |
| B       | 8                                                                    | AgBr/I   | 620                         | 100             |
| C       | 8                                                                    | AgBr/I   | 625-630                     | 190             |
| D       | 8                                                                    | AgBr/I   | 638                         | 153             |
| E       | 8                                                                    | AgBr/I   | 645                         | 224             |
| F       | 8                                                                    | AgBr/I   | 620                         | 196             |
| G       | 6                                                                    | AgBr/I   | 640                         | 62              |
| H       | 8                                                                    | AgBr/I   | 628                         | 200             |
| I       | 8                                                                    | AgBr/I   | 600                         | 59              |
| J       | 8                                                                    | AgBr/I   | 630                         | 112             |
| K       | 8                                                                    | AgBr/I   | 635                         | 210             |
| L       | 6                                                                    | AgBr/I   | 644                         | 435             |
| M       | 8                                                                    | AgBr/I   | 626                         | 230             |

Red sensitivity is shown as the relative sensitivity based on the red sensitivity of sensitizing dye B being 100 when exposed using Fuji No. 7 filter (red filter).

TABLE 3

| Dye No. | Amount of sensitizing dye (10 <sup>-5</sup> mols/kg. emulsion) (ml.) | Emulsion | Maximum sensitization (nm.) | Red sensitivity |
|---------|----------------------------------------------------------------------|----------|-----------------------------|-----------------|
| 1       | 8                                                                    | AgBr/I   | 664                         | 440             |
| 2       | 8                                                                    | AgBr/I   | 660                         | 294             |
| 3       | 8                                                                    | AgBr/I   | 632                         | 236             |
| 4       | 8                                                                    | AgBr/I   | 632                         | 141             |
| 5       | 3                                                                    | AgBr/I   | 632                         | 224             |
| 6       | 6                                                                    | AgBr/I   | 625                         | 147             |
| 7       | 8                                                                    | AgBr/I   | 636                         | 580             |
| 8       | 8                                                                    | AgBr/I   | 657                         | 253             |
| 9       | 8                                                                    | AgBr/I   | 670                         | 310             |
| 10      | 6                                                                    | AgBr/I   | 690                         | 470             |
| 11      | 8                                                                    | AgBr/I   | 660                         | 400             |

Red sensitivity is shown as the relative sensitivity based on the red sensitivity of sensitizing dye B being 100 when exposed using the Fuji No. 7 filter (red filter).

TABLE 4

| Example No. | Dye No. | Amount of dye (10 <sup>-3</sup> moles/kg. emulsion) (ml.) | Emulsion | Maximum sensitization (nm.) | Red sensitivity | 5  |
|-------------|---------|-----------------------------------------------------------|----------|-----------------------------|-----------------|----|
| 1.....      | A + 1   | 6 + 2                                                     | AgBr/I   | 634                         | 206             |    |
|             | B       | 8                                                         | AgBr/I   | 604                         | 440             |    |
|             | 4       | 8                                                         | AgBr/I   | 658                         | 550             |    |
| 2.....      | B + 4   | 5 + 3                                                     | AgBr/I   | 620                         | 100             |    |
|             | C       | 8                                                         | AgBr/I   | 632                         | 141             |    |
| 3.....      | C + 9   | 6 + 2                                                     | AgBr/I   | 640                         | 215             | 10 |
|             | D       | 8                                                         | AgBr/I   | 625-539                     | 190             |    |
|             | 5       | 6                                                         | AgBr/I   | 670                         | 310             |    |
|             | 10      | 8                                                         | AgBr/I   | 638                         | 153             |    |
| 4.....      | D + 5   | 6 + 2                                                     | AgBr/I   | 625                         | 147             |    |
| 5.....      | D + 10  | 4 + 4                                                     | AgBr/I   | 690                         | 470             |    |
|             | E       | 8                                                         | AgBr/I   | 684                         | 580             | 15 |
|             | 3       | 8                                                         | AgBr/I   | 645                         | 224             |    |
|             | 6       | 8                                                         | AgBr/I   | 632                         | 236             |    |
| 6.....      | E + 3   | 2 + 6                                                     | AgBr/I   | 636                         | 224             |    |
| 7.....      | E + 6   | 2 + 6                                                     | AgBr/I   | 645                         | 330             |    |
|             | G       | 6                                                         | AgBr/I   | 640                         | 380             |    |
|             | 2       | 8                                                         | AgBr/I   | 625                         | 62              |    |
| 8.....      | G + 2   | 2 + 6                                                     | AgBr/I   | 660                         | 294             | 20 |
|             | J       | 8                                                         | AgBr/I   | 630                         | 350             |    |
| 9.....      | J + 2   | 4 + 4                                                     | AgBr/I   | 650                         | 112             |    |
|             | L       | 6                                                         | AgBr/I   | 644                         | 350             |    |
| 10.....     | L + 2   | 4 + 4                                                     | AgBr/I   | 658                         | 435             |    |
|             | H       | 8                                                         | AgBr/I   | 628                         | 550             |    |
|             | I       | 8                                                         | AgBr/I   | 600                         | 200             |    |
|             | 7       | 8                                                         | AgBr/I   | 670                         | 59              |    |
| 11.....     | H + 7   | 1 + 7                                                     | AgBr/I   | 662                         | 580             | 25 |
| 12.....     | I + 7   | 1 + 7                                                     | AgBr/I   | 666                         | 700             |    |
|             | K       | 8                                                         | AgBr/I   | 635                         | 770             |    |
|             | F       | 8                                                         | AgBr/I   | 620                         | 210             |    |
| 13.....     | K + 2   | 4 + 4                                                     | AgBr/I   | 650                         | 196             |    |
| 14.....     | F + 2   | 2 + 6                                                     | AgBr/I   | 652                         | 355             | 30 |
|             | L       | 6                                                         | AgBr/I   | 644                         | 500             |    |
|             | 8       | 8                                                         | AgBr/I   | 657                         | 435             |    |
|             | 11      | 8                                                         | AgBr/I   | 660                         | 253             |    |
| 15.....     | L + 8   | 7 + 1                                                     | AgBr/I   | 640                         | 400             |    |
| 16.....     | L + 11  | 3 + 5                                                     | AgBr/I   | 658                         | 530             |    |
|             | M       | 8                                                         | AgBr/I   | 626                         | 535             |    |
|             | 2       | 8                                                         | AgBr/I   | 660                         | 230             |    |
| 17.....     | M + 2   | 4 + 4                                                     | AgBr/I   | 645                         | 294             |    |
|             |         |                                                           |          | 360                         | 35              |    |

Red sensitivity is shown as the relative sensitivity based on the red sensitivity of sensitizing dye B being 100 when exposed using the Fuji No. 7 filter (red filter).

As is clear from Table 4, it is understood that the red sensitivity increases remarkably when using combinations of sensitizing dyes (I) and (II) as compared with the cases of using the sensitizing dyes (I) and (II) by themselves.

What is claimed is:

1. A silver halide light-sensitive photographic emulsion containing a combination of at least one sensitizing dye represented by the following Formula I and at least one sensitizing dye represented by the following Formula II:



wherein  $\text{R}_1$  and  $\text{R}_2$  each represents a lower alkyl group or a substituted lower alkyl group,  $\text{Z}_1$  and  $\text{Z}_2$  each represents an atomic group necessary to complete a benzothiazole nucleus, a benzoselenazole nucleus or a naphthothiazole nucleus,  $\text{X}_1$  represents an anion, and  $n$  represents 0 or 1,  $n=0$  when an intra-molecular salt is formed;



wherein  $\text{R}_5$  represents a lower alkyl group and  $\text{R}_3$ ,  $\text{R}_4$ ,  $\text{Z}_3$ ,  $\text{Z}_4$ ,  $\text{X}_2$  and  $m$  each has the same meaning as  $\text{R}_1$ ,  $\text{R}_2$ ,  $\text{Z}_1$ ,  $\text{Z}_2$ ,  $\text{X}_1$  and  $n$ , respectively.

75

## 10

2. The silver halide light-sensitive photographic emulsion as claimed in claim 1 wherein said substituted alkyl group is a sulfo-containing alkyl group, a carboxy-containing alkyl group, a hydroxyalkyl group or an allyl group.

3. The silver halide light-sensitive photographic emulsion as claimed in claim 1 wherein sensitizing dye (I) is a compound selected from the group consisting of



11



12



and



4. The silver halide light-sensitive photographic emulsion as claimed in claim 1 wherein sensitizing dye (II) is a compound selected from the group consisting of



75

13



14

and



5. The silver halide light-sensitive photographic emulsion as claimed in claim 1 further comprising at least one pseudocyanine dye.

6. The silver halide light-sensitive photographic emulsion as claimed in claim 1 wherein the amount of each of said sensitizing dyes varies from  $10^{-6}$  mole to  $10^{-3}$  mole per mole of silver halide in said emulsion and wherein in the molar ratio of dye (I) to dye (II) varies from 9:1 to 1:9.

7. A light-sensitive photographic material comprising a support having coated thereon at least one layer containing the silver halide light-sensitive photographic emulsion as claimed in claim 1.

25

## References Cited

## UNITED STATES PATENTS

|           |         |                |       |        |
|-----------|---------|----------------|-------|--------|
| 2,422,080 | 6/1947  | Collins et al. | ----- | 96—124 |
| 2,533,427 | 12/1950 | Carroll        | ----- | 96—124 |
| 3,432,303 | 3/1969  | Jones et al.   | ----- | 96—124 |
| 3,617,293 | 11/1971 | Shiba et al.   | ----- | 96—124 |

J. TRAVIS BROWN, Primary Examiner

35

U.S. Cl. X.R.

96—137, 139

UNITED STATES PATENT OFFICE  
CERTIFICATE OF CORRECTION

Patent No. 3,677,765 Dated July 18, 1972

Inventor(s) Yoshiyuki Nakazawa et al

It is certified that error appears in the above-identified patent and that said Letters Patent are hereby corrected as shown below:

In The Heading:

The first inventor's last name is misspelled. Should read:

--Yoshiyuki Nakazawa. . . --

Signed and sealed this 10th day of July 1973.

(SEAL)

Attest:

EDWARD M.FLETCHER, JR.  
Attesting Officer

Rene Tegtmeier  
Acting Commissioner of Patents